# EUROPEAN PATENT SPECIFICATION

(11) **EP 3 705 608 B1**
(45) Date of publication and mention of the grant of the patent: **22.05.2024**
(21) Application number: 18873736.5
(22) Date of filing: 01.11.2018
(51) Int. Cl.: C25D 7/06, C25D 3/32, C25D 21/18, C25D 5/50

(54) **ELECTROLYTICALLY Sn-PLATED STEEL SHEET**
ELEKTROLYTISCH SN-PLATTIERTES STAHLBLECH
TÔLE D'ACIER PLAQUÉE DE SN PAR VOIE ÉLECTROLYTIQUE

(30) Priority: 01.11.2017 JP 2017211788
(43) Date of publication of application: 09.09.2020
(73) Proprietor: Nippon Steel Corporation, Tokyo 1008071 (JP)
(72) Inventor: GOTO, Yasuto, Tokyo 100-8071 (JP); TAJIMA, Yuta, Tokyo 100-8071 (JP); KOBAYASHI, Akinobu, Tokyo 100-8071 (JP)
(74) Representative: Vossius & Partner Patentanwälte Rechtsanwälte mbB
(86) International application number: PCT/JP2018/040727
(87) International publication number: WO 2019/088229

(56) References cited:
- JP-A- H03 191 097
- JP-A- 2005 314 750
- JP-A- 2006 519 311
- JP-A- 2017 523 300
- US-A1- 2010 216 302
- US-A1- 2013 183 542

## Description

### [Technical Field of the Invention]

The present invention relates to an electrolytic Sn-plated steel sheet, and particularly, to an electrolytic Sn-plated steel sheet having a low Pb content in a whole electrolytic Sn-plated layer.

### [Related Art]

In recent years, various regulations for Pb content in industrial products have been strengthened in view of concerns about health damage and measures against environmental loads.

The same also applies to a Sn-plated steel sheet (so-called tin can material) which is used for food canning. For example, in the Republic of South Africa, the Pb content in a Sn-plated layer is required to be 100 ppm by mass or less in view of the regulation of Pb²⁺ eluted in a can, and introduction of similar regulations has been considered in some European countries or in China. Demands similar to the above description have also been made from some customers.

In Japan, Sn ingots which are used for plating of a Sn-plated steel sheet are imported from Southeast Asian countries. Since the Pb content of the raw ore is large, the Sn ingots produced in Southeast Asia contain 100 ppm by mass or greater of Pb. In a case where the Sn ingots produced in Southeast Asia are used as they are, the Pb content in a Sn-plated layer of a Sn-plated steel sheet as a product cannot be adjusted to 100 ppm by mass or less. Accordingly, in a case where Sn ingots produced in Southeast Asia are used, electrolytic refining is performed even with an increase in the producing cost, to secure a level at which the current regulation value is somewhat satisfied. Otherwise, Sn ingots produced in South America, which have a small Pb content, are purchased even with an increase in the transport cost due to a long transport distance, to cope with the problems caused by the above regulation. In a case where tin is produced using Sn ingots produced in South America, the Pb content is about 70 ppm by mass, and this is at a level at which the current regulation value is somewhat satisfied.

In a case where an anode consisting of crude Sn produced from Sn ore or a Sn waste material is subjected to electrolytic refining, a part of Pb contained in the anode is dissolved as Pb²⁺ in the electrolytic solution, and in order to prevent the mixing of Pb in the electrolytic Sn occurring due to the above problem, Patent Document I describes an invention relating to an electrolytic refining method for high-purity Sn, in which a Sn electrolytic solution consisting of a fluorosilicic acid or a mixed acid of a sulfuric acid and a fluorosilicic acid is extracted from an electrolysis tank, a carbonate of an alkaline earth metal is added to the electrolytic solution to precipitate Pb in the solution, the electrolytic solution from which the precipitate is removed is returned to the electrolysis tank to perform electrolytic refining of Sn. However, Patent Document I has no description about the Pb content in a Sn-plated steel sheet and in a Sn-plated layer.

Patent Document 2 describes a technique in which a workpiece made of a pure metal or an alloy is heated and melted, and at least one of a metal halide or an oxyhalide is brought into contact with the melt to remove Pb in the workpiece. However, in Patent Document 2, only Pb-free solder is described as a specific workpiece, and there is no description about the Pb content in a Sn-plated layer of a Sn-plated steel sheet.

Patent Document 3 describes an invention in which an angle formed between adjacent grain boundaries in a Sn-plated layer is adjusted to 20° or less in order to prevent a short circuit between terminals due to the growth of whisker that is likely to occur in a case where Pb-free Sn plating is performed on an electronic component such as a semiconductor device. However, Patent Document 3 does not describe a method of producing Sn plating having an extremely low Pb concentration from a coating bath containing Pb.
US 2010/0216302 A1 discloses electrolyte compositions for depositing a tin alloy on a substrate.

### [Prior Art Document)

### [Patent Documents]

[Patent Document 1] Japanese Unexamined Patent Application, First Publication No. 2003-183871
[Patent Document 2] Japanese Unexamined Patent Application, First Publication No. 2010-111912
[Patent Document 3] Japanese Unexamined Patent Application, First Publication No. 2009-270154

### [Disclosure of the Invention]

### [Problems to be Solved by the Invention]

In view of the above situation and further strengthening of the Pb content regulation value that is anticipated, an object of the invention is to provide an electrolytic Sn-plated steel sheet which has a Pb content of 50 ppm by mass or less in a whole electrolytic Sn-plated layer and is applicable as a steel sheet for a container. More specifically, an object of the invention is to provide an electrolytic Sn-plated steel sheet which has a long life and has excellent corrosion resistance, coating film adhesion, and whisker resistance in a case where the steel sheet is applied as a steel sheet for a container.

### [Means for Solving the Problem]

The scope of the invention is stated in the claims.

### [Effects of the Invention]

According to the aspect of the invention, it is possible to provide an electrolytic Sn-plated steel sheet which has a Pb content of 50 ppm by mass or less in a whole electrolytic Sn-plated layer and is applicable as a steel sheet for a container.

### [Brief Description of the Drawings]

FIG. 1 is a graph showing changes in the Pb²⁺ concentration in a coating bath by a laboratory-scale crown ether method as an example of the invention.
FIG. 2A is a graph showing results of GD-MS analysis of an electrolytic Sn-plated layer of No. 16 of Example.
FIG. 2B is a graph showing changes in the value of Pb/(Sn+Pb) of No. 16 of Example in a thickness direction of the electrolytic Sn-plated layer.
FIG. 3A is a graph showing results of GD-MS analysis of an electrolytic Sn-plated layer produced using a Sn plating solution subjected to no treatment.
FIG. 3B is a graph showing results of GD-MS analysis of an electrolytic Sn-plated layer produced using a Sn plating solution treated by a crown ether method as an example of the invention.

### [Embodiments of the Invention]

Hereinafter, preferred embodiments of the invention will be described in detail. However, the invention is not limited to the configuration disclosed in this embodiment, and various modifications can be made within the scope of the amended claims.

Numerical limit ranges described below include the lower limit value and the upper limit value. Numeric values expressed by "greater than" or "less than" are not included in the numerical range.

An electrolytic Sn-plated steel sheet according to this embodiment includes: a base steel sheet; and an electrolytic Sn-plated layer which is disposed on the base steel sheet, has a Sn layer and an alloy layer, and contains Sn: 10 to 100 mass%, Fe: 0 to 90 mass%, and O: 0 to 0.5 mass%, the Pb content of the whole electrolytic Sn-plated layer is 50 ppm by mass or less, and in a case where the thickness of the electrolytic Sn-plated layer is represented by t and a region from a surface of the electrolytic Sn-plated layer to a depth of (1/10)×t in a sheet thickness direction is defined as a surface layer region, the Pb content of the surface layer region is 5 ppm by mass or greater and 60 ppm by mass or less and the Pb
content of the surface layer region is higher than the Pb content of the whole electrolytic Sn-plated layer.

First, the background to the development of the electrolytic Sn-plated steel sheet according to this embodiment by the inventors will be described.

The inventors have investigated the mechanism in which Pb contained in a Sn ingot is mixed in the electrolytic Sn-plated layer.

As a result of the investigation by the inventors, the inventors have found from the observation and quantitative measurement of the electrolytic Sn-plated layer in the depth direction that Pb exists as metal Pb in the whole electrolytic Sn-plated layer, that is, Pb is electrolytically deposited (eutectoid) together with Sn and is not contained in the electrolytic Sn-plated layer by mere involvement of a Sn plating solution.

The inventors prepared a Sn plating solution (PSA coating bath) including a p-phenolsulfonic acid, a Sn (II) sulfate, and additives, and a Pb-containing plating solution obtained by adding a Pb acetate to the Sn plating solution, and formed an electrolytic Sn-plated layer by changing a set potential. As a result, the inventors have found that there is almost no difference in the deposition potential between Sn and Pb, and that in a case where a Sn ingot having a low Pb content (about 50 ppm by mass) is used as a Sn source, the Pb content in the electrolytic Sn-plated layer can be adjusted to 100 ppm by mass or less (about 70 ppm by mass), and in a case where a Sn ingot having a high Pb content (about 100 to 300 ppm by mass) is used, it is difficult to suppress eutectoid of Pb by changing the plating conditions such as a current density with the use of the Sn plating solution which is used in an actual operation.

The Sn plating solution which is used in the plating step of the electrolytic Sn-plated steel sheet supplies Sn²⁺ in the form of a sulfuric acid bath using an insoluble anode, and the solubilities of the sulfates of Sn and Pb at 20°C are as follows.
SnSO₄: 18.9 g/100 g-H₂O(readily soluble)
PbSO₄: 0.003846 g/100 g-H₂O (hardly soluble)

It is thought that in the Sn plating solution in an actual operation, Pb²⁺ slightly dissolved as described above is electrically reduced together with Sn²⁺ and mixed as metal Pb in the electrolytic Sn-plated layer. The inventors have investigated the method of removing Pb²⁺ slightly dissolved as described above from the Sn plating solution, and as a result, found a removing method using a crown ether as a candidate.

A crown ether is formed of a cyclic polyether chain and can selectively interact with several heavy metal ions. A crown ether has a vacancy formed by ether oxygen atoms in the molecule, and takes in a heavy metal ion and binds therewith. Accordingly, a selective interaction occurs in a case where the size of the heavy metal ion and the size of the vacancy in the crown ether match. In order to selectively remove a lead ion (Pb²⁺) in the Sn plating solution, a crown ether in which the size of the vacancy is adjusted to match the size of the lead ion may be used.

For example, a crown ether in which in the general structural formula (-CH₂-CH₂-O-)ₙ of the crown ether, n is 6, and the size of a vacancy is controlled is supported on a resin (which is not particularly limited, and can be selected from, for example, silica gel, methacrylate, and polystyrene), a column is filled with the resin, and the Sn plating solution is allowed to pass through the column to selectively remove a lead ion (Pb²⁺).

Next, the inventors observed changes of Pb²⁺ in the Sn plating solution in the treatment of the Sn plating solution (PSA coating bath) with a crown ether in the laboratory scale.

The Sn plating solution as a base contains p-phenolsulfonic acid: 115 g/L, ethoxylated α-naphthol (EN-10): 5 g / L, ethoxylated α-naphthol sulphonic acid (ENSA): 5 g/L, and SnSO₄: 36 g/L (20 g/L in terms of Sn²⁺), and Pb is added to the Sn plating solution in the form of a Pb acetate such that Pb is contained at a concentration of 13 mg/L (650 ppm in terms of Pb/Sn) in terms of Pb²⁺.

A total of 200 L of the Sn plating solution was allowed to pass through a column filled with a crown ether, and component analysis was performed for each 20 L of the Sn plating solution passing through the column.

FIG. 1 shows changes in the Pb²⁺ concentration in the Sn plating solution.

As shown in FIG. 1, Pb²⁺ contained at a concentration of 13 mg/L is immediately reduced to 0.05 mg/L, and thus it is found that Pb²⁺ in the Sn coating bath is removed by the crown ether. Although not shown in the drawing, since the concentrations of other components (Sn²⁺, SO₄², ENSA, EN) in the Sn plating solution are hardly changed, it is thought that only Pb²⁺ is selectively removed.

In general, the uniformity in the electrolytic Sn-plated layer is increased in order to secure stable productivity. Accordingly, the Pb content in the electrolytic Sn-plated layer is uniformly reduced in the depth direction. However, the inventors have newly found that unlike the prior art, the occurrence of staining is reduced by reducing the Pb content of the whole electrolytic Sn-plated layer, and whisker resistance is improved by concentrating Pb in the surface layer region. In addition, the inventors have also newly found that coating film adhesion is improved by imparting a gradient to the Pb content in the electrolytic Sn-plated layer.

The electrolytic Sn-plated steel sheet according to this embodiment is provided based on the above knowledge. Hereinafter, the electrolytic Sn-plated steel sheet according to this embodiment will be described in detail.

### [Base Steel Sheet]

A base steel sheet of the electrolytic Sn-plated steel sheet according to this embodiment is not particularly limited, and a steel sheet which is used as a base steel sheet of a general steel sheet for a container specified in JIS G 3303: 2017 may be used. In this embodiment, for example, a base steel sheet containing C: 0.01 to 0.06 mass%, A1: 0.001 to 0.01 mass%, Mn: 0.01 to 0.06 mass%, and the remainder consisting of Fe and impurities can be used.

### [Electrolytic Sn-Plated Layer]

An electrolytic Sn-plated layer according to this embodiment has a Sn layer existing on the surface side of the electrolytic Sn-plated layer and containing a large amount of Sn, and an alloy layer (Fe-Sn layer) existing on the base steel sheet side of the electrolytic Sn-plated layer, in which Fe of the base steel sheet is diffused in the electrolytic Sn-plated layer. The definitions of the electrolytic Sn-plated layer, the Sn layer, and the alloy layer will be described later.

In this embodiment, the Pb content of the whole electrolytic Sn-plated layer is 50 ppm by mass or less. In a case where the Pb content of the whole electrolytic Sn-plated layer is greater than 50 ppm by mass, the Pb content regulation value that is anticipated cannot be satisfied, and characteristics (long life, corrosion resistance) desired for a steel sheet for a container cannot be obtained. The Pb content of the whole electrolytic Sn-plated layer is preferably 40 ppm by mass or less, 30 ppm by mass or less, 20 ppm by mass or less, or 10 ppm by mass or less. Although it is possible to make the Pb content of the whole electrolytic Sn-plated layer less than 5 ppm by mass, this causes a cost increase in an actual operation. Accordingly, the lower limit of the Pb content of the whole electrolytic Sn-plated layer may be set to 5 ppm by mass.

In the electrolytic Sn-plated layer according to this embodiment, the Pb content of the surface layer region is 5 ppm by mass or greater, and the Pb content of the surface layer region is higher than the Pb content of the whole electrolytic Sn-plated layer. The upper limit of the Pb content of the surface layer region is 60 ppm by mass. In this embodiment, the surface layer region refers to a region from a surface of the electrolytic Sn-plated layer to a depth of (1/10)×t in a sheet thickness direction, in a case where the thickness of the electrolytic Sn-plated layer is represented by t. In this embodiment, a region other than the surface layer region of the electrolytic Sn-plated layer is referred to as a deep region. That is, the deep region of the electrolytic Sn-plated layer is a region ranging from the region from the depth of (1/10)×t from the surface of the electrolytic Sn-plated layer in the sheet thickness direction to the depth t in the sheet thickness direction from the surface, in a case where the thickness of the electrolytic Sn-plated layer is represented by t.

In a case where the Pb content of the surface layer region is equal to the Pb content of the whole electrolytic Sn-plated layer, or the Pb content of the surface layer region is lower than the Pb content of the whole electrolytic Sn-plated layer, the coating film adhesion of the electrolytic Sn-plated steel sheet deteriorates.

In the electrolytic Sn-plated layer according to this embodiment, a value obtained by dividing (Pb content/(Sn content+Pb content)) of the surface layer region of the electrolytic Sn-plated layer by (Pb content/(Sn content+Pb content)) of the deep region of the electrolytic Sn-plated layer may be 1.1 or greater. In a case where the value obtained by dividing (Pb content/(Sn content+Pb content)) of the surface layer region of the electrolytic Sn-plated layer by (Pb content/(Sn content+Pb content)) of the deep region of the electrolytic Sn-plated layer is 1.1 or greater, the coating film adhesion of the electrolytic Sn-plated steel sheet can be further improved.

The electrolytic Sn-plated layer according to this embodiment contains Sn: 10 to 100 mass%, Fe: 0 to 90 mass%, and O: 0 to 0.5 mass% as elements other than Pb. The remainder consists of impurities. In this embodiment, the impurities mean elements which are mixed from the Sn ingot as a raw material or the producing environment, and are permitted within a range not adversely affecting the electrolytic Sn-plated steel sheet according to this embodiment.

The electrolytic Sn-plated layer according to this embodiment may further optionally contain one or more of the group consisting of Ca: 0.1 to 10 ppm by mass, Sr: 0.1 to 10 ppm by mass, and Ba: 0.1 to 10 ppm by mass. The Pb content of the whole electrolytic Sn-plated layer can be further reduced in a case where the electrolytic Sn-plated layer contains one or more of the above group.

The electrolytic Sn-plated steel sheet according to this embodiment may further include one or more of a Fe-Ni layer, a Ni-Sn layer, and a Fe-Ni-Sn layer between the electrolytic Sn-plated layer and the base steel sheet, strictly speaking, between the alloy layer (Fe-Sn layer) and the base steel sheet. In a case where the electrolytic Sn-plated layer further includes one or more of these layers, the can life can be extended in a case where the electrolytic Sn-plated steel sheet is used as a beverage can or a food can. In addition, since a barrier effect is generated due to the formation of a dense alloy layer, corrosion resistance can be improved.

Next, a method of analyzing the components of the electrolytic Sn-plated layer according to this embodiment will be described with reference to FIGS. 2A and 2B. The components of the electrolytic Sn-plated layer can be analyzed by glow dischargemass spectrometry (GD-MS) analysis. The GD-MS analysis is an analysis method of tracking changes of the composition of the plated layer from the surface in the depth direction with the lapse of the discharge time. FIG. 2A is a graph obtained by performing GD-MS analysis on an electrolytic Sn-plated steel sheet of No. 16 of Example.

The graph of FIG. 2A shows changes in the contents of Fe, Sn, Pb, and O from the surface side of the electrolytic Sn-plated layer on the left end side of the horizontal axis toward the base steel sheet side on the right end side. Regarding the ppm by mass on the vertical axis, the scale on the left side is for Fe and Sn, and the scale on the right side is for Pb and O.

The graph of FIG. 2B is obtained by acquiring the Sn content and the Pb content of FIG. 2A, calculating a value of Pb/(Sn+Pb), and making changes in the depth direction from the surface of the electrolytic Sn-plated layer into a graph.

In this embodiment, in the GD-MS analysis in the sheet thickness direction of a sample collected from an arbitrary position in the electrolytic Sn-plated steel sheet, a region ranging from the surface to a region having a Sn content of 100,000 ppm or greater is defined as the electrolytic Sn-plated layer. In FIG. 2A, no element is detected for several minutes after discharge, and this region is not included in the electrolytic Sn-plated layer. In the electrolytic Sn-plated layer, a region where the Sn content is higher than the Fe content is defined as a Sn layer, and in the electrolytic Sn-plated layer, a region other than the Sn layer is defined as an alloy layer (Fe-Sn layer) (see FIG. 2A). A region where the Fe content is 10 to 90 mass% and the Ni content is 10 to 90 mass% is defined as a Fe-Ni layer, a region where the Ni content is 10 to 90 mass% and the Sn content is 10 to 90 mass% is defined as a Ni-Sn layer, and a region where the Fe content is 10 to 80 mass%, the Ni content is 10 to 80 mass%, and the Sn content is 10 to 80 mass% is defined as a Fe-Ni-Sn layer.

The Pb content of the whole electrolytic Sn-plated layer is the Pb content of the whole electrolytic Sn-plated layer including the Sn layer and the alloy layer, obtained by GD-MS analysis. The Pb content of the surface layer region is the Pb content of a region from the surface of the electrolytic Sn-plated layer to a depth of (1/10)×t, obtained by GD-MS analysis.

(Pb content/(Sn content+Pb content)) of the surface layer region of the electrolytic Sn-plated layer is obtained by dividing the Pb content (mass%) of the surface layer region by the sum of the Sn content (mass%) and the Pb content (mass%) of the surface layer region. Similarly, (Pb content/(Sn content+Pb content)) of the deep region of the electrolytic Sn-plated layer is obtained by dividing the Pb content (mass%) of the deep region by the sum of the Sn content (mass%) and the Pb content (mass%) of the deep region.

The Ca content, the Sr content, and the Ba content in the electrolytic Sn-plated layer are obtained by analyzing a solution, obtained by dissolving the electrolytic Sn-plated layer using an acid containing an inhibitor, by inductively coupled plasma-mass spectrometry (ICP-MS).

### [Producing Method]

An example of the method of producing the electrolytic Sn-plated steel sheet according to this embodiment will be described.

First, electrolytic Sn plating is applied to the base steel sheet having the above-described chemical composition. In this embodiment, electrolytic Sn plating is performed using a Sn plating solution having a Pb²⁺ concentration reduced by a crown ether method. Electrolytic degreasing may be performed before the electrolytic Sn plating. In the electrolytic Sn plating step in which sheet threading is performed at a high speed between a plurality of electrodes (10 passes), the current density of the first to ninth passes is made constant, and the current density of the 10th pass (final pass) is increased to perform the electrolytic Sn plating. The Pb content of the surface layer region of the electrolytic Sn-plated layer can be adjusted by adjusting the increase width of the current density of the 10th pass. After the electrolytic Sn plating step, flux coating is performed on the base steel sheet, followed by immersion in a 10-fold dilution of the Sn plating solution. After roller squeezing, cold air drying is performed, and energization heating and quenching (80°C) are performed as a reflow operation.

Through the above method, the electrolytic Sn-plated steel sheet according to this embodiment can be produced.

In this embodiment, a carbonate of an alkaline earth metal (Ca, Sr, Ba) may be added to the Sn plating solution. Accordingly, the yield of Pb²⁺ removal by the crown ether method can be improved, and the Pb content of the whole electrolytic Sn-plated layer can be further reduced.

In this embodiment, Ni pre-plating or Fe-Ni pre-plating may be performed as a pretreatment for electrolytic Sn plating. Accordingly, one or more of a Fe-Ni layer, a Ni-Sn layer, and a Fe-Ni-Sn layer can be formed between the base steel sheet and the electrolytic Sn-plated layer.

### [Examples]

Hereinafter, Examples of the invention will be described below. However, conditions in Examples are merely examples employed for confirming the practicability and effects of the invention, and the invention is not limited to these condition examples. The invention can employ various conditions as long as the object of the invention is achieved without departing from the gist of the invention.

### [Example 1]

The effect of reduction in the Pb content in an electrolytic Sn-plated layer by a crown ether method was investigated in the actual operation scale.

Components of a Sn plating solution were as follows: Sn²⁺: 20 g/L; Pb²⁺: 5 mg/L (250 ppm in terms of Pb/Sn); EN: 5 g/L; ENSA: 5 g/L; and PSA: 100 g/L, and the temperature was 45°C.

A column was filled with a resin on which a crown ether had been supported (silica gel was used in this Example), and the Sn plating solution was allowed to pass through the column. The Sn plating solution was moved to a plating cell, and returned to the column after circulation in the plating cell. The above operation was repeated. In this case, as a result of preliminary investigation, a flow rate (L/hr) of the Sn plating solution was set to 60 L/hr for 1 L of the resin although depending on a resin volume (L).

Although a considerable effect was recognized in the laboratory scale, Pb²⁺ was reduced only to 0.1 mg/L in the actual operation scale.

The inventors have presumed that this is because the characteristics of the crown ether slightly deteriorate due to the presence of a large amount of pre-existing sludge (containing SnO₂ as a main component) in the actual operation line. However, it has been found that the effect can be sufficiently exhibited even in the actual operation line by adjusting the flow rate or the exchange frequency of the crown ether.

An electrolytic Sn-plated layer produced using a Sn plating solution in which Pb²⁺ had been reduced by a crown ether method was analyzed.

FIG. 3B shows results of GD-MS analysis of an electrolytic Sn-plated layer produced using a Sn plating solution which contains Pb²⁺: 0.1 mg/L through the crown ether method. FIG. 3A shows results of GD-MS analysis of an electrolytic Sn-plated layer (comparative example) produced using a Sn plating solution subjected to no treatment.

As shown in FIG. 3A, from the electrolytic Sn-plated layer as a comparative example produced using the Sn plating solution subjected to no treatment, a high concentration of Pb was detected together with Sn from the vicinity of the surface. From the plated layer produced using the Sn plating solution treated by the crown ether method, only a slight amount of Pb was detected as shown in FIG. 3B.

### [Example 2]

The following experiment was conducted on the assumption that the electrolytic Sn-plated steel sheet according to the invention was applied to the production of tin as a beverage can material or a food can material.

A steel sheet containing C: 0.03 mass%, Al: 0.005 mass%, Mn: 0.03 mass%, and the remainder consisting of Fe and impurities was used as a base steel sheet.

Components of a Sn plating solution were as follows: Sn²⁺: 20 g/L; Pb²⁺: 5 mg/L (250 ppm in terms of Pb/Sn); EN: 5 g/L; ENSA: 5 g/L; and PSA: 100 g/L, and the temperature was 45°C. The Pb²⁺ concentration of the Sn plating solution was reduced by a crown ether method, and an electrolytic Sn-plated layer was sequentially formed at an arbitrary Pb²⁺ concentration through an electrolytic Sn plating step to be described later. It was possible to reduce the Pb²⁺ concentration down to 0.05 mg/L in the laboratory scale.

As a pretreatment for forming the electrolytic Sn-plated layer, an electrolytic degreasing step of the steel sheet was performed in which a current of 10 A/dm²×10 sec was allowed to flow such that the steel sheet was on the cathode side in a 10% NaOH solution at 60°C. Then, pickling was performed by dipping in 10% H₂SO₄ at room temperature for 10 seconds, and then electrolytic Sn plating was performed at 5 A/dm² using the above Sn plating solution to achieve #25 tin (adhered amount of Sn on single side: 2.8 g/m²).

In the electrolytic Sn plating step, in this Example, the current density of the final pass among the 10 passes was changed, and thus an electrolytic Sn-plated layer in which the distribution state of Pb was controlled was formed. That is, the current density of the final pass was increased to concentrate Pb in a surface layer region, and conversely, the current density of the final pass was reduced to make the Pb content of the surface layer region lower than the Pb content of the whole electrolytic Sn-plated layer. In this Example, the current density was maintained at 20 A/dm² except for the final pass, and increased to 30 to 60 A/dm² in the final pass, and the electrolytic Sn plating was performed. However, in cases of No. 11 and No. 14 of Table 1, only the current density of the final pass was reduced, and in cases of No. 37 and No. 38, the current density was made constant.

A carbonate of an alkaline earth metal (Ca, Sr, Ba) was added to some Sn plating solutions.

After the electrolytic Sn plating step, flux coating was performed, followed by immersion in a 10-fold dilution of the above-described electrolytic Sn plating solution. After roller squeezing, cold air drying was performed, and energization heating and quenching (80°C) were performed as a reflow operation. Through the above method, an electrolytic Sn-plated steel sheet was obtained.

For some electrolytic Sn-plated steel sheets, Ni pre-plating or Fe-20 mass% Ni pre-plating was performed as a pretreatment for the electrolytic Sn plating step such that the adhered amount of Ni was 20 mg/m². Then, a Fe-Ni layer, a Ni-Sn layer (mainly containing Ni₃Sn₄), or a Fe-Ni-Sn layer was formed by reflow.

Component analysis of the electrolytic Sn-plated layer was performed by the above-described method. For GD-MS analysis, a rectangular sample of 30 mm×15 mm was collected from a position 30 mm away from an end portion of the electrolytic Sn-plated steel sheet, and the GD-MS analysis was performed at two positions in the sample. Trace element analysis of alkaline earth metals (Ca, Sr, Ba) was performed by ICP-MS. The electrolytic Sn-plated layer contains Pb, Ca, Sr, and Ba shown in Table 1, and contains Sn: 10 to 100 mass%, Fe: 0 to 90 mass%, O: 0 to 0.5 mass%, and the remainder consisting of impurities.

"Pb Content in Whole Plated Layer/ppm by mass" in Table 1 represents the Pb content of the whole electrolytic Sn-plated layer, and "Pb content of Surface Layer/ppm by mass" represents the Pb content of the surface layer region of the electrolytic Sn-plated layer. In the column of "Pb/(Sn+Pb) (surface layer region/deep region)" in Table 1, the symbol "O" is indicated in a case where a value obtained by dividing (Pb content/(Sn content+Pb content)) of the surface layer region of the electrolytic Sn-plated layer by (Pb content/(Sn content+Pb content)) of the region (deep region) other than the surface layer region of the electrolytic Sn-plated layer is 1.1 or greater, and the symbol "×" is indicated in a case where the value is less than 1.1.

In Table 1, all Examples including invention examples and comparative examples had a Sn layer and an alloy layer in the electrolytic Sn-plated layer.

The following tests were performed on the electrolytic Sn-plated steel sheet.

In a sulfide staining resistance test (retort test), a sample having a predetermined size was collected from a position 30 mm away from an end portion of the electrolytic Sn-plated steel sheet, and a current was allowed to flow to the sample at 5 A/dm² by using a Pb-Sn anode in a 25 g/L solution of sodium dichromate dihydrate at 50°C to achieve 10 mg/dm² (#311 treatment).

### Alloy-Tin Couple Test (ATC Test)

The can life in a case where the electrolytic Sn-plated steel sheet was applied to a beverage can or a food can was evaluated by an ATC test. In the ATC test, an electrolytic Sn-plated steel sheet detinned after reflow, in which an alloy layer (Fe-Sn layer) was exposed, and an electrolytic Sn-plated steel sheet which had not been detinned after reflow were immersed in an ATC test solution (1.5% NaCl+ 1.5% citric acid solution), and a corrosion current flowing between the two electrodes was measured. A rectangular test piece of 130 mm×15 mm was prepared. The test piece was subjected to electrolytic peeling in a 5% NaOH solution, and a surface other than a test surface of 5 mm×40 mm was completely sealed to prevent leakage of the current. The test solution was boiled for 2 minutes in a nitrogen atmosphere and cooled to room temperature. The electrolytic Sn-plated steel sheet detinned after reflow, in which the alloy layer (Fe-Sn layer) was exposed, and the electrolytic Sn-plated steel sheet which had not been detinned after reflow were connected and incorporated in a test tank. Stannous chloride (100 ppm in terms of Sn²⁺) was added to the bottom of the test tank to previously put the inside of the test tank in a nitrogen atmosphere. The ATC test solution was moved to the test tank so as not to come into contact with air. The electrolytic Sn-plated steel sheet detinned after reflow, in which the alloy layer (Fe-Sn layer) was exposed, and the electrolytic Sn-plated steel sheet which had not been detinned after reflow were immersed, and at the same time, the ATC test solution was stirred for 30 minutes to dissolve the stannous chloride. After immersion in the nitrogen atmosphere (ATC test solution) for 20 hours, a current value between the detinned electrolytic Sn-plated steel sheet and the electrolytic Sn-plated steel sheet which had not been detinned was measured, and was set as an ATC value. The lower the ATC value, the longer the can life.

In this Example, scores were given depending on the ATC value (µA/cm²) measured by the above method in four stages of:
Excellent 4 Points: less than 0.1 µA/cm²
   3 points: 0.1 µA/cm² or greater and less than 0.2 µA/cm²
   2 points: 0.2 µA/cm² or greater and less than 0.3 µA/cm²
Poor 1 point: 0.3 µA/cm² or greater
Since it was possible to use an electrolytic Sn-plated steel sheet with a score of 2 or greater as a steel sheet for a container, a score of 2 or greater was determined to be acceptable.

### Sulfide Staining Resistance Test (retort test)

The corrosion resistance of the electrolytic Sn-plated steel sheet was evaluated by a sulfide staining resistance test. In the sulfide staining resistance test, a corrosion resistance test solution in which a 0.1% sodium thiosulfate aqueous solution and a 0.1 N sulfuric acid were mixed at a volume fraction of 1:2 was used. The electrolytic Sn-plated steel sheet subjected to the above-described #311 treatment was cut into a ϕ35 mm piece and prepared as a test piece. The test piece was placed and fixed on the mouth of a heat-resistant bottle containing a corrosion resistance test solution. Then, the heat-resistant bottle was turned upside down such that the test piece and the corrosion resistance test solution were brought into contact with each other. A heat treatment was performed for 60 minutes at 121°C, and then corrosion resistance was evaluated based on a ratio of the corroded portion in the area where the corrosion resistance test solution was brought into contact with the test piece (the area of the opening part of the heat-resistant bottle).

Scores from 1 to 5 points were given depending on the ratio of the corrosion area to the area where the corrosion resistance test solution was brought into contact with the test piece. Since it was possible to use an electrolytic Sn-plated steel sheet with a score of 3 or greater as a steel sheet for a container, a score of 3 or greater was determined to be acceptable.
Excellent 5 Points: area of less than 10%
   4 Points: area of 10% or greater and less than 25%
   3 Points: area of 25% or greater and less than 40%
   2 Points: area of 40% or greater and less than 55%
Poor 1 Point: area of 55% or greater

### Coating Film Adhesion Evaluation Test

A sample was collected from an arbitrary position in the electrolytic Sn-plated steel sheet. An acrylic coating film was coated on the surface of the electrolytic Sn-plated layer by baking, cooled to room temperature, and then subjected to a tape peeling test. The tape surface after the peeling test was observed, and a case where a surface to which the electrolytic Sn plating was adhered was less than 5% of the tape surface (the surface where the electrolytic Sn-plated layer and the tape were adhered to each other) was determined to be acceptable as excellent coating film adhesion. A case where the surface to which the electrolytic Sn plating was adhered was 5% or greater of the tape surface (the surface where the electrolytic Sn-plated layer and the tape were adhered to each other) was determined to be unacceptable as poor coating film adhesion. Among the examples determined to be acceptable, a case where the surface to which the electrolytic Sn plating was adhered was less than 3% of the tape surface (the surface where the electrolytic Sn-plated layer and the tape were adhered to each other) was determined to be particularly excellent coating film adhesion. In Table 1, the symbol "Δ" was indicated for the examples determined to be acceptable. Among the examples determined to be acceptable, those having excellent coating film adhesion were indicated by the symbol "O", and those determined to be unacceptable were indicated by the symbol "x".

### Whisker Resistance Evaluation Test

A sample was collected from an arbitrary position in the electrolytic Sn-plated steel sheet. The sample was subjected to 5 T-bending and left for 1,000 h at 40°C and 50%RH. Then, the outside of the bent portion was observed in the range of 10 mm×5 mm by SEM, and the number of whiskers of 50 µm or greater was counted by observing 3 visual fields. The number was divided by the observation area to obtain a number density. A case where the number of observed whiskers was 10 or less per 1 mm² was determined to be acceptable as excellent whisker resistance, and a case where the number of observed whiskers was greater than 10 was determined to be unacceptable. In Table 1, the symbol "O" was indicated for the examples determined to be acceptable, and the symbol "×" was indicated for the examples determined to be unacceptable.

The measurement results and test results are shown in Table 1. In Table 1, the underline indicates that the characteristic is out of the scope of the invention or not preferred.

**[Table 1]**

| | Pb Content in Whole Plated Layer/ppm by mass | Pb content of Surface Layer/ppm by mass | Pb/(Sn+Pb) (surface layer region/deep region) | Content in Plated Layer/ppm by mass | | | Pre-Plating | ATC Score | Sulfide Staining Resistance Score | Coating Film Adhesion Evaluation | Whisker Resistance Evaluation | Remarks |
|---|---|---|---|---|---|---|---|---|---|---|---|---|
| | | | | Ca | Sr | Ba | | | | | | |
| No. 1 | 210 | 215 | ○ | - | - | - | - | 1 | 1 | ○ | ○ | Comparative Example |
| No.2 | 110 | 112 | ○ | - | - | - | - | 1 | 1 | ○ | ○ | Comparative Example |
| No.3 | 70 | 75 | ○ | - | - | - | - | 1 | 2 | ○ | ○ | Comparative Example |
| No.4 | 48 | 58 | ○ | - | - | - | - | 3 | 3 | ○ | ○ | Invention Example |
| No.5 | 39 | 43 | ○ | - | - | - | - | 3 | 3 | ○ | ○ | Invention Example |
| No.6 | 30 | 32 | × | - | - | - | - | 3 | 4 | Δ | ○ | Invention Example |
| No.7 | 19 | 23 | ○ | - | - | - | - | 4 | 5 | ○ | ○ | Invention Example |
| No.8 | 9 | 12 | ○ | - | - | - | - | 4 | 5 | ○ | ○ | Invention Example |
| No.9 | 49 | 60 | ○ | - | - | - | - | 3 | 3 | ○ | ○ | Invention Example |
| No.10 | 49 | 50 | × | - | - | - | - | 2 | 3 | Δ | ○ | Invention Example |
| No.11 | 48 | 40 | × | - | - | - | - | 2 | 3 | × | ○ | Comparative Example |
| No.12 | 29 | 42 | ○ | - | - | - | - | 4 | 3 | ○ | ○ | Invention Example |
| No.13 | 28 | 30 | × | - | - | - | - | 3 | 4 | Δ | ○ | Invention Example |
| No.14 | 28 | 24 | × | - | - | - | - | 3 | 4 | × | ○ | Comparative Example |
| No.15 | 16 | 28 | ○ | - | - | - | - | 4 | 4 | ○ | ○ | Invention Example |
| No.16 | 15 | 25 | ○ | - | - | - | - | 4 | 5 | ○ | ○ | Invention Example |
| No.17 | 15 | 20 | ○ | - | - | - | - | 4 | 5 | ○ | ○ | Invention Example |
| No.18 | 15 | 16 | × | - | - | - | - | 4 | 5 | Δ | ○ | Invention Example |
| No.19 | 38 | 49 | ○ | 0.1 | - | - | - | 3 | 3 | ○ | ○ | Invention Example |
| No.20 | 38 | 49 | ○ | 0.5 | - | - | - | 3 | 3 | ○ | ○ | Invention Example |
| No.21 | 38 | 49 | ○ | 1 | - | - | - | 3 | 3 | ○ | ○ | Invention Example |
| No.22 | 38 | 49 | ○ | 4 | - | - | - | 3 | 3 | ○ | ○ | Invention Example |
| No.23 | 38 | 49 | ○ | 8 | - | - | - | 3 | 3 | ○ | ○ | Invention Example |
| No.24 | 32 | 42 | ○ | - | 0.2 | - | - | 4 | 4 | ○ | ○ | Invention Example |
| No.25 | 31 | 40 | ○ | - | 0.5 | - | - | 4 | 4 | ○ | ○ | Invention Example |
| No.26 | 33 | 43 | ○ | - | 1 | - | - | 4 | 4 | ○ | ○ | Invention Example |
| No.27 | 31 | 40 | ○ | - | 5 | - | - | 4 | 4 | ○ | ○ | Invention Example |
| No.28 | 32 | 42 | ○ | - | 10 | - | - | 4 | 4 | ○ | ○ | Invention Example |
| No.29 | 45 | 59 | ○ | - | - | 0.1 | - | 3 | 3 | ○ | ○ | Invention Example |
| No .30 | 44 | 57 | ○ | - | - | 0.5 | - | 3 | 3 | ○ | ○ | Invention Example |
| No.31 | 42 | 55 | ○ | - | - | 1 | - | 3 | 3 | ○ | ○ | Invention Example |
| No.32 | 43 | 56 | ○ | - | - | 4 | - | 3 | 3 | ○ | ○ | Invention Example |
| No.33 | 44 | 57 | ○ | - | - | 7 | - | 3 | 3 | ○ | ○ | Invention Example |
| No.34 | 32 | 42 | ○ | 2 | 1 | - | - | 4 | 4 | ○ | ○ | Invention Example |
| No.35 | 48 | 59 | ○ | - | - | - | Ni | 4 | 3 | ○ | ○ | Invention Example |
| No.36 | 48 | 59 | ○ | - | - | - | Fe-20%Ni | 4 | 3 | ○ | ○ | Invention Example |
| No.37 | 48 | 48 | × | - | - | - | Ni | 3 | 3 | × | ○ | Comparative Example |
| No.38 | 48 | 48 | × | - | - | - | Fe-20%Ni | 3 | 3 | × | ○ | Comparative Example |
| No.39 | 5 | 7 | ○ | - | - | - | - | 5 | 5 | ○ | ○ | Invention Example |
| No.40 | 2 | 3 | ○ | - | - | - | - | 5 | 5 | ○ | × | Comparative Example |

No. 1, No. 2, and No. 3 are examples in which the Pb content of the whole electrolytic Sn-plated layer was greater than 50 ppm by mass, and the scores of the ATC test and the sulfide staining resistance test were low. Sulfide staining is caused by binding of Sn and S, and discoloration is promoted by exposition to a high temperature in the retort treatment. It is presumed that in a case where the Pb content of the whole electrolytic Sn-plated layer is high, a portion where the melting point is lowered is locally generated, the number of reaction points of discoloration is increased, and thereby this leads to an appearance change called macro staining.

In the invention examples, the Pb content of the whole electrolytic Sn-plated layer is 50 ppm by mass or less, and the Pb content of the surface layer region is 5 ppm or greater and is higher than the Pb content of the whole electrolytic Sn-plated layer. Accordingly, all the results of the ATC test, the sulfide staining resistance test, the coating film adhesion evaluation test, and the whisker resistance evaluation test were good.

Specifically, more favorable corrosion resistance was exhibited in a case where the Pb content of the whole electrolytic Sn-plated layer was 30 ppm by mass or less (No. 6), and extremely favorable corrosion resistance was exhibited in a case where the Pb content of the whole electrolytic Sn-plated layer was 20 ppm by mass or less (No. 7, No. 8, and Nos. 16 to 18). In addition, the invention examples in which the value obtained by dividing (Pb content/(Sn content+Pb content)) of the surface layer region of the electrolytic Sn-plated layer by (Pb content/(Sn content+Pb content)) of the deep region of the electrolytic Sn-plated layer was 1.1 or greater exhibited particularly good results in the coating film adhesion evaluation test.

Nos. 19 to 23 are electrolytic Sn-plated steel sheets produced by adding 0.01 to 1g/L of calcium carbonate to the Sn plating solution corresponding to No. 10. The Pb content of the whole electrolytic Sn-plated layer in Nos. 19 to 23 was reduced by about 20% as compared to No. 10, and this indicated an improvement in the Pb²⁺ yield by the crown ether method.

Nos. 24 to 28 are electrolytic Sn-plated steel sheets produced by adding 0.01 to 1g/L of strontium carbonate to the Sn plating solution corresponding to No. 10. The Pb content of the whole electrolytic Sn-plated layer in Nos. 24 to 28 was reduced by about 30% as compared to No. 10, and this indicated an improvement in the Pb²⁺ yield by the crown ether method.

Nos. 29 to 33 are electrolytic Sn-plated steel sheets produced by adding 0.01 to 1g/L of barium carbonate to the Sn plating solution corresponding to No. 10. The Pb content of the whole electrolytic Sn-plated layer in Nos. 29 to 33 was reduced by about 10% as compared to No. 10, and this indicated an improvement in the Pb²⁺ yield by the crown ether method.

No. 34 is an electrolytic Sn-plated steel sheet produced by adding 0.07 g/L of calcium carbonate and 0.05 g/L of strontium carbonate to the Sn plating solution corresponding to No. 10. The Pb content of the whole electrolytic Sn-plated layer in No. 34 was reduced by about 35% as compared to No. 10, and this indicated an improvement in the Pb²⁺ yield by the crown ether method.

Nos. 35 to 38 are examples in which pre-Ni plating and pre-Fe-20% Ni plating were performed prior to electrolytic Sn plating corresponding to No. 9. In No. 35 and No. 36 as the invention examples, one or more of a Ni-Fe layer, a Ni-Sn layer, and a Ni-Fe-Sn layer were formed. Accordingly, it has been found that the potential difference between the electrolytic Sn-plated layer and the Ni-Fe layer, Ni-Sn layer, or Ni-Fe-Sn layer was reduced and the ATC value was improved.

FIGS. 2A and 2B show the results of GD-MS analysis of the electrolytic Sn-plated layer after a reflow treatment of the electrolytic Sn-plated steel sheet produced in the Example (No. 16).

The graph of FIG. 2A shows changes in the content ratios of Fe, Sn, Pb, and O from the surface of the electrolytic Sn-plated layer on the left end side of the horizontal axis toward the base steel sheet on the right end side of the horizontal axis. Regarding the ppm by mass on the vertical axis, the scale on the left side is for Fe and Sn, and the scale on the right side is for Pb and O. From FIG. 2A, it is found that only about 25 ppm by mass of Pb is detected in the outermost surface.

The graph of FIG. 2B is obtained by acquiring the Sn content and the Pb content of FIG. 2A, calculating a value of Pb/(Sn+Pb), and making changes in the depth direction from the surface of the electrolytic Sn-plated layer into a graph.

In this case, it is found that the value of Pb/(Sn+Pb) is increased in the surface layer region of the electrolytic Sn-plated layer (the region from the surface to a depth of (1/10)×t in the sheet thickness direction (the portion surrounded by a rectangle in FIG. 2B)), that is, a Pb concentration phenomenon occurs near the surface.

In the example of FIG. 2B, the average value of Pb/(Sn+Pb) in the whole electrolytic Sn-plated layer was about 15 ppm by mass, whereas the maximum value of Pb/(Sn+Pb) in the surface layer region was about 25 ppm by mass and was below the current Pb content regulation value that is anticipated. There was no substantial problem.

In a case where the Pb content in the whole electrolytic Sn-plated layer reaches the upper limit value of 50 ppm by mass specified in the invention, the upper limit value of the Pb content in the surface layer region is 60 ppm by mass.

In the invention, an electrolytic Sn-plated steel sheet having a low Pb content is obtained by a complex formation/capture/removal method of Pb²⁺ ions with a crown ether in order to reduce the Pb content of a whole electrolytic Sn-plated layer. However, the invention does not exclude the use of a method other than the complex formation/capture/removal method of Pb²⁺ ions with a crown ether.

### [Industrial Applicability]

According to this embodiment, it is possible to provide an electrolytic Sn-plated steel sheet which has a Pb content of 50 ppm by mass or less in a whole electrolytic Sn-plated layer and is applicable as a steel sheet for a container. According to this embodiment, without the use of a high-cost Sn ingot having a low Pb content, it is possible to achieve a low Pb content at low cost while using a conventional Sn ingot having a relatively high Pb content produced in Southeast Asia or the like. Therefore, even in a case where regulations such as achieving a Pb-free state are strengthened all over the world, the invention can deal with the above situation, and has great meaningfulness in the industry.

## Claims

1. An electrolytic Sn-plated steel sheet comprising:
a base steel sheet; and
an electrolytic Sn-plated layer which is disposed on the base steel sheet, has a Sn layer and an alloy layer, and contains Sn: 10 to 100 mass%, Fe: 0 to 90 mass%, and O: 0 to 0.5 mass%, wherein the Sn layer exists on the surface side of the electrolytic Sn-plated layer and the alloy layer exists on the base steel sheet side of the electrolytic Sn-plated layer,
wherein a Pb content of the whole electrolytic Sn-plated layer is 50 ppm by mass or less, and
in a case where a thickness of the electrolytic Sn-plated layer is represented by t and a region from a surface of the electrolytic Sn-plated layer to a depth of (1/10)×t in a sheet thickness direction is defined as a surface layer region, a Pb content of the surface layer region is 5 ppm by mass or greater and 60 ppm by mass or less and the Pb content of the surface layer region is higher than the Pb content of the whole electrolytic Sn-plated layer, wherein the components of the electrolytic Sn-plated layer is analyzed by glow dischargemass spectrometry (GD-MS) analysis,
in the GD-MS analysis in the sheet thickness direction of a sample collected from an arbitrary position in the electrolytic Sn-plated steel sheet, a region ranging from the surface to a region having a Sn content of 100,000 ppm or greater is defined as the electrolytic Sn-plated layer while a region wherein no element is detected for several minutes after discharge is not included in the electrolytic Sn-plated layer,
in the electrolytic Sn-plated layer, a region where the Sn content is higher than the Fe content is defined as a Sn layer, and in the electrolytic Sn-plated layer, a region other than the Sn layer is defined as an alloy layer (Fe-Sn layer).

2. The electrolytic Sn-plated steel sheet according to claim 1,
wherein a value obtained by dividing (Pb content/(Sn content+Pb content)) of the surface layer region of the electrolytic Sn-plated layer by (Pb content/(Sn content+Pb content)) of a region other than the surface layer region of the electrolytic Sn-plated layer is 1.1 or greater.

3. The electrolytic Sn-plated steel sheet according to claim 1 or 2,
wherein the electrolytic Sn-plated layer further contains one or more of the group consisting of Ca: 0.1 to 10 ppm by mass, Sr: 0.1 to 10 ppm by mass, and Ba: 0.1 to 10 ppm by mass.

4. The electrolytic Sn-plated steel sheet according to any one of claims 1 to 3, further comprising:
one or more of a Fe-Ni layer, a Ni-Sn layer, and a Fe-Ni-Sn layer between the electrolytic Sn-plated layer and the base steel sheet,
wherein a region where the Fe content is 10 to 90 mass% and the Ni content is 10 to 90 mass% is defined as a Fe-Ni layer, a region where the Ni content is 10 to 90 mass% and the Sn content is 10 to 90 mass% is defined as a Ni-Sn layer, and a region where the Fe content is 10 to 80 mass%, the Ni content is 10 to 80 mass%, and the Sn content is 10 to 80 mass% is defined as a Fe-Ni-Sn layer.

## Patentansprüche

1. Ein elektrolytisch Sn-plattiertes Stahlblech, umfassend:
ein Grundstahlblech; und
eine elektrolytisch Sn-plattierte Schicht, welche auf dem Grundstahlblech bereitgestellt ist, eine Sn-Schicht und eine Legierungsschicht aufweist und Sn: 10 bis 100 Massen-%, Fe: 0 bis 90 Massen-% und O: 0 bis 0,5 Massen-% enthält, wobei die Sn-Schicht auf der Oberflächenseite der elektrolytisch Sn-plattierten Schicht vorhanden ist und die Legierungsschicht auf der Seite des Grundstahlblechs der elektrolytisch Sn-plattierten Schicht vorhanden ist,
wobei ein Pb-Gehalt der gesamten elektrolytisch Sn-plattierten Schicht 50 Massen-ppm oder weniger beträgt und
in einem Fall, in welchem eine Dicke der elektrolytisch Sn-plattierten Schicht durch t dargestellt wird und ein Bereich von einer Oberfläche der elektrolytisch Sn-plattierten Schicht zu einer Tiefe von (1/10)×t in einer Blechdickenrichtung als ein Oberflächenschichtbereich definiert ist, ein Pb-Gehalt des Oberflächenschichtbereichs 5 Massen-ppm oder größer und 60 Massen-ppm oder weniger beträgt und der Pb-Gehalt des Oberflächenschichtbereichs höher als der Pb-Gehalt der gesamten elektrolytisch Sn-plattierten Schicht ist, wobei die Komponenten der elektrolytisch Sn-plattierten Schicht mittels Glimmentladungs-Massenspektrometrieanalyse (GD-MS) analysiert werden,
in der GD-MS-Analyse in der Blechdickenrichtung einer Probe, welche an einer beliebigen Position in dem elektrolytisch Sn-plattierten Stahlblech gesammelt wurde, ein Bereich, welcher sich von der Oberfläche zu einem Bereich mit einem Sn-Gehalt von 100,000 ppm oder größer erstreckt, als die elektrolytisch Sn-plattierte Schicht definiert ist, während ein Bereich, in dem mehrere Minuten nach der Entladung kein Element zu erkennen ist, nicht in der elektrolytischen Sn-Schicht enthalten ist,
in der elektrolytisch Sn-plattierten Schicht, ein Bereich, in welchem der Sn-Gehalt höher ist als der Fe-Gehalt, als eine Sn-Schicht definiert ist, und in der elektrolytisch Sn-plattierten Schicht, ein anderer Bereich als der der Sn-Schicht als eine Legierungsschicht (Fe-Sn-Schicht) definiert ist.

2. Das elektrolytisch Sn-plattierte Stahlblech gemäß Anspruch 1,
wobei ein Wert, der durch Dividieren von (Pb-Gehalt/(Sn-Gehalt+Pb-Gehalt)) des Oberflächenschichtbereichs der elektrolytisch Sn-plattierten Schicht durch (Pb-Gehalt/(Sn-Gehalt+Pb-Gehalt)) eines anderen Bereichs als des Oberflächenschichtbereichs der elektrolytisch Sn-plattierten Schicht erhalten wird, 1,1 oder größer ist.

3. Das elektrolytisch Sn-plattierte Stahlblech gemäß Anspruch 1 oder 2,
wobei die elektrolytisch Sn-plattierte Schicht ferner eines oder mehrere der Gruppe bestehend aus Ca: 0,1 bis 10 Massen-ppm, Sr: 0,1 bis 10 Massen-ppm und Ba: 0,1 bis 10 Massen-ppm enthält.

4. Das elektrolytisch Sn-plattierte Stahlblech gemäß einem der Ansprüche 1 bis 3, ferner umfassend:
eines oder mehrere einer Fe-Ni-Schicht, einer Ni-Sn-Schicht und einer Fe-Ni-Sn-Schicht zwischen der elektrolytisch Sn-plattierten Schicht und dem Grundstahlblech,
wobei ein Bereich, in welchem der Fe-Gehalt 10 bis 90 Massen-% und der Ni-Gehalt 10 bis 90 Massen-% beträgt, als eine Fe-Ni-Schicht definiert ist, ein Bereich, in welchem der Ni-Gehalt 10 bis 90 Massen-% und der Sn-Gehalt 10 bis 90 Massen-% beträgt, als eine Ni-Sn-Schicht definiert ist und ein Bereich, in welchem der Fe-Gehalt 10 bis 80 Massen-%, der Ni-Gehalt 10 bis 80 Massen-% und der Sn-Gehalt 10 bis 80 Massen-% beträgt, als eine Fe-Ni-Sn-Schicht definiert ist.

## Revendications

1. Tôle d'acier plaquée de Sn par voie électrolytique, comprenant :
une tôle d'acier de base ; et
une couche plaquée de Sn par voie électrolytique qui est disposée sur la tôle d'acier de base, a une couche de Sn et une couche d'alliage, et contient Sn : 10 à 100 % en masse, Fe : 0 à 90 % en masse, et O : 0 à 0,5 % en masse, dans laquelle la couche de Sn existe sur le côté surface de la couche plaquée de Sn par voie électrolytique et la couche d'alliage existe sur le côté tôle d'acier de base de la couche plaquée de Sn par voie électrolytique,
dans laquelle la teneur en Pb de la couche plaquée de Sn par voie électrolytique est de 50 ppm en masse ou moins, et
dans le cas où l'épaisseur de la couche plaquée de Sn par voie électrolytique est représentée par t et la région allant d'une surface de la couche plaquée de Sn par voie électrolytique jusqu'à une profondeur de (1/10)×t dans la direction de l'épaisseur de la tôle est définie comme étant une région de couche de surface, la teneur en Pb de la région de couche de surface est de 5 ppm en masse ou plus et 60 ppm en masse ou moins, et la teneur en Pb de la région de couche de surface est supérieure à la teneur en Pb de toute la couche plaquée de Sn par voie électrolytique, dans laquelle les composants de la couche plaquée de Sn par voie électrolytique sont analysés par une analyse par spectrométrie de masse à décharge luminescente (GD-MS),
dans l'analyse GD-MS dans la direction de l'épaisseur de la tôle d'un échantillon collecté à partir d'une position arbitraire dans la tôle d'acier plaquée de Sn par voie électrolytique, une région allant de la surface à une région ayant une teneur en Sn de 100 000 ppm ou plus est définie comme étant la couche plaquée de Sn par voie électrolytique tandis qu'une région dans laquelle aucun élément n'est détecté pendant plusieurs minutes après une décharge n'est pas incluse dans la couche plaquée de Sn par voie électrolytique,
dans la couche plaquée de Sn par voie électrolytique, une région dans laquelle la teneur en Sn est supérieure à la teneur en Fe est définie comme étant une couche de Sn, et dans la couche plaquée de Sn par voie électrolytique, une région autre que la couche de Sn est définie comme étant une couche d'alliage (couche de Fe-Sn).

2. Tôle d'acier plaquée de Sn par voie électrolytique selon la revendication 1, dans laquelle une valeur obtenue en divisant (teneur en Pb / (teneur en Sn + teneur en Pb)) de la région de couche de surface de la couche plaquée de Sn par voie électrolytique par (teneur en Pb / (teneur en Sn + teneur en Pb)) d'une région autre que la région de couche de surface de la couche plaquée de Sn par voie électrolytique est de 1,1 ou plus.

3. Tôle d'acier plaquée de Sn par voie électrolytique selon la revendication 1 ou 2, dans laquelle la couche plaquée de Sn par voie électrolytique contient en outre un ou plusieurs du groupe consistant en Ca : 0,1 à 10 ppm en masse, Sr : 0,1 à 10 ppm en masse, et Ba : 0,1 à 10 ppm en masse.

4. Tôle d'acier plaquée de Sn par voie électrolytique selon l'une quelconque des revendications 1 à 3, comprenant en outre :
une ou plusieurs parmi une couche de Fe-Ni, une couche de Ni-Sn, et une couche de Fe-Ni-Sn entre la couche plaquée de Sn par voie électrolytique et la tôle d'acier de base,
dans laquelle une région dans laquelle la teneur en Fe est de 10 à 90 % en masse et la teneur en Ni est de 10 à 90 % en masse est définie comme étant une couche de Fe-Ni, une région dans laquelle la teneur en Ni est de 10 à 90 % en masse et la teneur en Sn est de 10 à 90 % en masse est définie comme étant une couche de Ni-Sn, et une région dans laquelle la teneur en Fe est de 10 à 80 % en masse, la teneur en Ni est de 10 à 80 % en masse et la teneur en Sn est de 10 à 80 % en masse est définie comme étant une couche de Fe-Ni-Sn.
